

## UNITED STATES PATENT OFFICE

2,220,714

## PRODUCTION OF ASPHALT

Arthur B. Hersberger, Philadelphia, Pa., assignor  
to The Atlantic Refining Company, Philadelphia, Pa., a corporation of Pennsylvania

No Drawing. Application June 14, 1938,  
Serial No. 213,623

9 Claims. (Cl. 196—74)

The present invention relates to the treatment of bituminous materials, and particularly bituminous materials, such as cracked or uncracked petroleum residuum.

5 A principal object of this invention is the production of improved asphalts from bituminous residues, and particularly from petroleum residuum containing about 10% or less by weight of asphaltenes, which will not yield homogeneous asphalts when treated according to conventional methods.

10 A further object of this invention is the production of homogeneous asphalts having a negative Oliensis test from domestic crude petroleum residuum having a relatively low content of asphaltenes. Such test is described in A.S.T.M. Proceedings, part II, vol. 39 (1936), page 506 et seq., and is being widely adopted in asphalt specifications as an index of homogeneity of asphalt products.

15 20 A further object of this invention is the treatment of residuums produced by the cracking or non-cracking distillation of petroleum; residues from the hydrogenation of petroleum; heavy residual oils produced by polymerization; and residues produced by the treatment of petroleum oils with selective solvents or with asphalt-precipitating agents such as petroleum naphtha, pentane, butane, propane, ethane and the like.

25 30 In the production of asphalts, it has heretofore been customary to subject asphaltic crude oils to fire and steam distillation whereby volatile oils are removed, leaving an asphaltic residuum, or to subject the asphaltic residuum so produced to oxidation with air at elevated temperatures to yield asphalts of increased softening point. However, it has been found impossible to produce from petroleum residuums containing less than about 10% by weight of asphaltenes, satisfactory asphalts exhibiting a negative Oliensis test, by air oxidation, distillation or blending, or combination of such steps.

35 40 I have found that by treating bituminous materials, and particularly petroleum residuum, with sulfur and air or oxygen-containing gas at elevated temperatures such that reaction of the sulfur and air with the petroleum residuum is effected, I am able to obtain asphaltic materials of markedly increased softening point.

45 50 Furthermore, in accordance with my invention I am able to produce homogeneous asphalts, as indicated by a negative Oliensis test, from petroleum residuums which will not produce such asphalts when processed in the conventional manner. In other words, petroleum residuums which

5 cannot be converted into homogeneous asphalts by conventional distillation, air blowing, and blending or combination of such steps are amenable to my treatment and will yield homogeneous asphalts of the character of those derived from asphaltic crude oils such as Mexican and Venezuelan.

10 In carrying out my invention, a bituminous material such as a crude petroleum residuum is subjected to the action of sulfur, in the presence of an oxygen-containing gas such as air, at elevated temperatures of the order of from about 300° F. to about 550° F. for a period of time varying from about 1/2 hour to about 8 to 10 hours or more, depending upon the rate of reaction between the sulfur and air and the petroleum residuum. The quantity of sulfur employed may vary from about 0.5% to about 5% by weight, and is preferably of the order of from about 1% to about 3% by weight of the residuum treated. In 20 general, upwards of 95% of the quantity of sulfur brought into contact with the petroleum residuum is caused to react therewith.

15 25 Treatment of the residuum may be effected at substantially atmospheric pressure by simply blowing an oxygen-containing gas, such as air, through a mass of the residuum containing added sulfur at elevated temperatures, or the sulfur may be admixed with the residuum and treated with air at elevated temperatures and under a substantial superatmospheric pressure of the order of 30 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850

subjected to further treatment involving distillation and blending with oils or residues of different nature, preferably those rich in resins, i. e., containing 30% to 50% or more, of resins, will 5 produce homogeneous asphalts of the general character of those derived from the true asphaltic crude oils of Mexico and Venezuela. Petroleum residual oils, such as those resulting from the distillation of Texas, Oklahoma or other non-asphalt base crudes, cannot be converted into asphalts having a negative Oliensis test and the characteristics of Mexican or Venezuelan asphalts by merely blowing with air at elevated temperatures and distilling and blending the air-blown 10 products with other oils or residues.

The principal advantage of my process is the ability to produce, from domestic crude petroleum or petroleum deficient in asphaltenes, specification asphalts which are more homogeneous, as 15 measured by the Oliensis test, than asphalts produced from the same residuum by conventional methods of air oxidation, distillation and/or blending. A negative Oliensis test indicates a homogeneous asphalt, while a positive test indicates a non-homogeneous asphalt.

My invention may be illustrated by the following examples, which are not to be construed as limiting the scope thereof.

(1) A crude petroleum residuum (17% bottoms 20 from West Texas crude oil) having a Saybolt Universal viscosity of 839 seconds at 210° F., an A. P. I. gravity 12.5°, a flash point of 560° F., a fire point of 640° F., and comprising 52.5% oil, 44.0% resins, and 3.5% asphaltenes was blown with air, 25 in the absence of added sulfur, at a temperature of 400° F. for a period of 4 hours, air being supplied at a rate of 2.1 cubic feet/hour/gallon of residuum. As a result of such treatment there was produced an asphaltic material having a 30 softening point of 124° F., and a positive Oliensis test, which indicated the material to be non-homogeneous. The treated asphaltic material, when blended with untreated residuum in the ratio of 62 parts by weight to 28 parts by weight, 35 yielded a non-homogeneous asphalt having a positive Oliensis test.

A quantity of the same untreated residuum as employed above, to which had been added 2% by weight of sulfur, was blown with air under the 40 conditions as described above, and there was produced an asphaltic material having a softening point of 124° F., and a negative Oliensis test, which indicated the material to be homogeneous. This asphaltic material was then reduced to 150° F. 45 softening point by vacuum distillation, and the 150° F. softening point residue was blended in the ratio of 62 parts by weight to 38 parts by weight with the initial, untreated residuum. The resulting blended asphalt had a softening point 50 of 117° F., and a negative Oliensis test, indicating that the blended material was homogeneous. The other properties of this asphalt were substantially the same as those of an asphalt produced by fire and steam distillation of a Venezuelan crude oil.

(2) A quantity of the untreated residuum of Example 1, to which had been added 1% by weight of sulfur, was blown with air at a temperature of 400° F. for a period of 3 hours, air being supplied at a rate of 2.1 cubic feet/hour/gallon of residuum. 55 As a result of such treatment there was produced an asphaltic material having a softening point of 120° F., and a negative Oliensis test. This asphaltic material was blended in the ratio of 62 parts by weight to 38 parts by weight with the initial, untreated residuum, and the blended ma-

terial was then reduced by vacuum distillation, about 25% of volatile oils being removed. The resulting asphalt had a softening point of 115° F. and a negative Oliensis test. This asphalt also corresponded to a Venezuelan asphalt of the same 6 softening point.

(3) A naphthenic residual oil, produced by nitrobenzene extraction of West Texas crude residuum, having a Saybolt Universal viscosity of 1692 seconds at 210° F. and an A. P. I. gravity of 9.3°, 10 was admixed with 1.75% by weight of sulfur and the mixture was blown with air at a temperature of 400° F. for a period of 3 1/2 hours, air being supplied at a rate of 2.1 cubic feet/hour/gallon of residual oil. There was produced, as a result of 15 such treatment, an asphaltic material having a softening point of 126° F., and a negative Oliensis test. This asphaltic material was then blended in the ratio of 85 parts by weight to 15 parts by 20 weight of the initial, untreated residual oil and there resulted an asphalt having a softening point of 118° F., and a negative Oliensis test, said asphalt being similar in other properties to a Venezuelan asphalt of the same softening point.

(4) A quantity of the same untreated petroleum residuum as employed in Example 1 was admixed with 1% by weight of sulfur and the mixture was heated at a temperature of 450° F. under air pressure of 95 lbs./sq. in. for a period of 2 hours. As a result of such treatment there was 25 produced an asphalt having a softening point of 148° F., and a negative Oliensis test.

The same petroleum residuum, when treated under the same conditions, but in the absence of 30 added sulfur, yielded an asphaltic material having a softening point of 144° F., and a positive Oliensis test.

It will be seen from the above examples, that treatment of petroleum residuum at elevated temperatures with air and sulfur produces asphaltic 40 materials having a negative Oliensis test, which materials, when blended with residuum rich in resins, yield asphalts homogeneous in character, as evidenced by the negative Oliensis test. On the other hand, the same residuum, when merely air 45 blown at elevated temperatures but in the absence of added sulfur, yields asphaltic material which is non-homogeneous according to the Oliensis test. By my process involving treatment of petroleum residuum poor in asphaltenes with 50 air and sulfur at elevated temperatures, followed by distillation and/or blending with heavy oils rich in resins, there may be produced homogeneous asphalts having the general characteristics of steam refined Mexican or Venezuelan asphalts, 55 whereas such treatment in the absence of added sulfur will not produce the desired asphalts.

What I claim is:

1. The method of producing asphalt from petroleum residual oil containing less than about 60 10% of asphaltenes, which comprises contacting said residual oil with sulfur and free-oxygen containing gas at an elevated temperature such that reaction of the sulfur and free-oxygen containing gas with the residual oil is effected, and blending 65 the treated residual oil with high boiling hydrocarbon oil rich in resins.

2. The method of producing asphalt from petroleum residual oil containing less than about 70 10% of asphaltenes, which comprises contacting said residual oil with sulfur and free-oxygen containing gas at an elevated temperature such that reaction of the sulfur and free-oxygen containing gas with the residual oil is effected, removing from 75 the treated residual oil volatile oils, and blending 75

the residue with high boiling hydrocarbon oil rich in resins.

3. The method of producing asphalt from petroleum residual oil containing less than about 5 10% of asphaltenes, which comprises contacting said residual oil with sulfur and free-oxygen containing gas at a temperature of from about 300° F. to about 550° F. to cause reaction of the sulfur and free-oxygen containing gas with the residual 10 oil, removing from the treated residual oil volatile oils, and blending the residue with high boiling hydrocarbon oil rich in resins.

4. The method of producing asphalt from petroleum residual oil containing less than about 15 10% of asphaltenes, which comprises contacting said residual oil with from about 1% to about 3% by weight of sulfur and free-oxygen containing gas at a temperature of from about 300° F. to about 550° F. to cause reaction of the sulfur and 20 free-oxygen containing gas with the residual oil, removing from the treated residual oil volatile oils, and blending the residue with high boiling hydrocarbon oil rich in resins.

5. The method of producing asphalt having a 25 negative Oliensis test from petroleum residual oil containing less than about 10% of asphaltenes, which comprises contacting said residual oil with sulfur and air at an elevated temperature such that reaction of the sulfur and air with the residual oil is effected, and blending the treated 30 residual oil with high boiling hydrocarbon oil rich in resins.

6. The method of producing asphalt having a negative Oliensis test from petroleum residual oil 35 containing less than about 10% of asphaltenes, which comprises contacting said residual oil with sulfur and air at an elevated temperature such

that reaction of the sulfur and air with the residual oil is effected, removing from the treated residual oil volatile oils, and blending the residue with high boiling hydrocarbon oil rich in resins.

7. The method of producing asphalt having a 5 negative Oliensis test from petroleum residual oil containing less than about 10% of asphaltenes, which comprises contacting said residual oil with sulfur and air at a temperature of from about 300° F. to about 550° F. to cause reaction of the 10 sulfur and air with the residual oil, removing from the treated residual oil volatile oils, and blending the residue with high boiling hydrocarbon oil rich in resins.

8. The method of producing asphalt having a 15 negative Oliensis test from petroleum residual oil containing less than about 10% of asphaltenes, which comprises contacting said residual oil with from about 1% to about 3% by weight of sulfur and air at a temperature of from about 300° F. 20 to about 550° F. to cause reaction of the sulfur and air with the residual oil, removing from the treated residual oil volatile oils, and blending the residue with high boiling hydrocarbon oil rich 25 in resins.

9. The method of producing asphalt from petroleum residual oil containing less than about 10% of asphaltenes, which comprises contacting said residual oil with sulfur and air at a temperature of from about 300° F. to about 550° F. 30 to cause reaction of the sulfur and air with the residual oil, blending with said treated residual oil a quantity of oil rich in resins, and removing volatile oils from the blended material by distillation. 35

ARTHUR B. HERZBERGER.